

July 28, 1970

CHISATO KAWAZOE ET AL  
METHOD OF MANUFACTURING ELECTRIC CONDUCTOR  
INSULATED BY FOAMED CRYSTALLINE POLYMER  
Filed June 29, 1966

3,522,088

Fig. 1  
PRIOR ART



Fig. 2



INVENTORS  
CHISATO KAWAZOE, TERUMICHI ICHIBA,  
SEICHI IWAKURA & HIROSHI SHIMBA  
BY

CAROTHERS & CAROTHERS

THEIR ATTORNEYS

**1****3,522,088****METHOD OF MANUFACTURING ELECTRIC CONDUCTOR INSULATED BY FOAMED CRYSTALLINE POLYMER**

Chisato Kawazoe, Tokyo-to, Terumichi Ichiba, Kamakura-shi, and Seichi Iwakura and Hiroshi Shimba, Yokohama-shi, Japan, assignors to Sumitomo Electric Industries, Ltd., Osaka, Japan, a company of Japan

Filed June 29, 1966, Ser. No. 561,564

Claims priority, application Japan, July 7, 1965,  
40/40,727

Int. Cl. B44c 1/36, 1/42; C08f 29/04

U.S. Cl. 117—232

**1 Claim****ABSTRACT OF THE DISCLOSURE**

A method of manufacturing an electric conductor with a coating of a foamed polymer wherein the conductor is coated with a solvent solution of either polythene or polypropylene and dried to cause particle aggregation of the polymer which is physically noted by the clouding of the coating and to remove the solvent remaining. The dried coated conductor is then immersed in a liquid of monoatomic or polyatomic alcohol and heated to a temperature which is at least equal to the melting point of the selected polymer to cause foaming. The foamed coating is then rinsed in water to remove the residual alcohol and cool the coating.

The present invention relates to an improvement in the manufacture of foamed plastic insulated electric conductors of the type which have a high-temperature viscous solution of crystalline polymer, e.g. polythene or polypropylene, applied thereover which is thereafter treated to provide closed cells in the interior of coating.

Referring to the prior art illustration of FIG. 1, the conventional method employed for the manufacture of foamed plastic insulated electric conductors is conducted by first coating a viscous solution of crystalline polymer, e.g. polyethylene or polypropylene, over the conductor W in a solution coating tank 1. Then the coated conductor passes through a drying duct 3, which has its interior exposed to the atmosphere, for drying, followed by passing through a foaming furnace (or heating furnace) 4 to produce closed cells in the interior of the coating, and the foamed plastic insulated electric conductor thus obtained is taken up on a reel 5.

In the above-mentioned method, an electric furnace has been used for the foaming furnace 4 in which air or other incombustible gases are heated by electricity. When the conductor coated with a viscous solution of crystalline polymer passes through such an electric furnace as described above, the coated conductor is heated mainly by high temperature air or other incombustible gases and is partly heated by the heat radiation from the wall of the electric furnace. Thus, closed cells are obtained in the interior of the coating of coated conductor.

However, the heat capacity of air (or other incombustible gases) is small and furthermore the thermal conductivity of air (or other incombustible gases) is low, so that the high heating temperatures and long durations of heating are required for foaming. For instance, it takes approximately 4 seconds to obtain a coating with an expansion degree of 20-30% by passing the coated conductor through an electric furnace in which air is heated to 360° C.

Recently, it has been required to increase the line speed of coating machines for the purpose of increasing output. In order to increase the line speed by using the conventional foaming furnace, it is necessary to increase the length of the foaming furnace. As a result of this, the dis-

**2**

tance between supporting points of the coated conductor passing through the foaming furnace becomes longer, so that the coated conductor vibrates excessively at higher line speeds and consequently can cause damage to the coating. Furthermore, it is difficult to uniformly maintain the temperature distribution of gas in the cross-sectional and longitudinal directions of the furnace. In consequence, it is not easy to obtain a uniform foaming of the coating in its radial direction. When a number of coated conductors are placed in the furnace at the same time, it is furthermore not easy to obtain uniformity of the expansion state among the foamed conductors.

The object of the present invention is to provide a method of manufacturing foamed plastic insulated electric conductors, which makes it possible to shorten the time required to foam the interior of the coating and to obtain a uniformly foamed coating. The present invention is characterized in that after the viscous solution of crystalline polymer is coated over a conductor 20 and the coated conductor thus obtained is dried, the coated conductor is dipped in a heated liquid which hardly swells and dissolves said coating in order to foam the interior thereof (referred to as the melting point of the polymer). It is then rinsed and cooled with hot water or cold water, or both.

FIG. 2 is a block diagram showing the features of the manufacturing method of the present invention. Identical numerals and letters denote similar items.

After a viscous solution of crystalline polymer is coated 30 over the conductor W in the solution coating tank 1 and the coated conductor thus obtained is dried in the drying duct 3 as described in conjunction with FIG. 1. The coated conductor is dipped in the heated liquid trough 6 for foaming and is then rinsed and cooled in the water trough 7, followed by take-up on a reel 5.

For the heated liquid employed for foaming, any liquid which hardly swells the coating of crystalline polymer can be used. As a result of many experiments performed repeatedly, however, monoatomic or polyatomic 40 alcohols are preferable. Alcohols which may be used as the heating liquid, one may use ethylene glycol, diethylene glycol, tri-ethylene glycol, propylene glycol, butylene glycol, pentanediol, hexanediol, glycerin, etc. These alcohols scarcely swell and dissolve the coating of crystalline polymer, and can be readily rinsed out with water.

As for the temperature of the heating liquid, any temperature which is not lower than the melting point of the crystalline polymer employed in the coating and which is lower than the boiling point of the heating liquid is 50 acceptable. For example, the range of preferable temperature of the heating liquid is 120° C. to 250° C. when a viscous solution of high density polyethylene is used as the coating solution and glycerin is adopted as the heating liquid.

As one example of this invention, a 28 wt. percent solution of high density polythene in xylene, which was kept at approximately 130° C., was coated to 0.55 mm. in over-all diameter over a 0.32 mm. copper conductor and then the coating was dried. Foaming was then performed 60 on three different lengths of coated conductor by immersion in a glycerin bath at a temperature of 180° C. for 0.2 second, 0.5 second and 1 second respectively. The expansion degree of the coatings of these three electric conductor insulated by foamed polyethylene was measured. 65 As a result of the measurements, it has been ascertained that the expansion degree of 20-30% having been obtained with each of these three kinds was no different from those that were foamed by heating in an electric foaming furnace for about 4 seconds by use of the conventional method.

The above-mentioned manufacturing method by the present invention has the following advantages:

(1) Compared with the method hitherto employed in which a heating furnace, such as an electric furnace, is used and a coated conductor is heated by the heated air (or other incombustible gas) in the interior of the furnace and by heat radiation from the wall of the furnace, the method of the present invention in which a heating liquid is used, enjoys a greater heat capacity and heat transfer effect, so that it is possible to remarkably shorten the heating. It also makes it possible to employ a lower heating temperature for foaming.

(2) As the duration of heating is short, it is possible to shorten the length of the heating trough for foaming. This results in reduction of the distance between supporting points of the coated conductor. In addition, there is almost no chance in causing damage to the coating because the vibration of coated conductor in a liquid is much less than in a gas due to the damping effect of liquid.

(3) As the heating liquid used for foaming is compatible with water, it is easy to remove the residual liquid, which remains on the surface of the insulated conductor after foaming, with water.

(4) As the heat capacity and thermal conductivity of liquids are greater than those of gas, it is easy to obtain a much more uniform temperature distribution and temperature control throughout the heated liquid trough. This results in obtaining a more uniformly foamed coating of crystalline polymer.

What we claim is:

1. The method of manufacturing an electric conductor with a coating of a foamed polymer comprising the steps of coating the conductor with a solvent solution of a crystalline polymer selected from the group consisting of polythene and polypropylene, drying the coated conductor, immersing the dried coated conductor for not more than one second in a liquid selected from at least one in the group consisting of monoatomic alcohol and polyatomic alcohol and heated to a temperature of at least equal to the melting point of the selected polymer to cause foaming in the coating, and thereafter rinsing the foamed coated conductor with water to remove the residual liquid and cool the foamed coating.

#### References Cited

#### UNITED STATES PATENTS

|           |         |                 |       |           |
|-----------|---------|-----------------|-------|-----------|
| 3,121,760 | 2/1964  | Kline           | ----- | 264—51    |
| 3,170,968 | 2/1965  | Rokunohe et al. | ----- | 117—232   |
| 3,275,720 | 9/1966  | Ohsol           | ----- | 264—53    |
| 3,068,126 | 12/1962 | Rokunohe et al. | ----- | 117—232   |
| 3,154,605 | 10/1964 | Meyer et al.    | ----- | 117—119.6 |

WILLIAM D. MARTIN, Primary Examiner

R. M. SPEER, Assistant Examiner

U.S. CL. X.R.

117—119.8